

## UNITED STATES PATENT OFFICE

2,151,312

## HAMMERED METAL FINISH

Guido Ariotti, Stamford, Conn., assignor to Atlas Powder Company, Wilmington, Del., a corporation of Delaware

No Drawing. Application March 26, 1937,  
Serial No. 133,184

10 Claims. (Cl. 91—68)

This invention relates to a new method of finishing surfaces in simulation of hammered metal and to a composition for use in producing such finishes.

In the decoration of metallic surfaces, it has in the past been conventional to produce a hammered effect thereon by hammering the entire exposed surface of the metal with a round headed hammer or by means of a suitable machine producing the same effect. The effect produced is well known and comprises innumerable depressed portions over the surface of the metal. This method is tedious and expensive. Moreover, it can be produced only on metal surfaces and preferably those which are of soft metal. The metal base must be of substantial thickness in order to withstand the hammering and to yield the desired effect. Consequently, it is desirable to have available a simple method by which there may be applied to any base a coating material which will, when dry, yield a surface which simulates hammered metal in appearance.

This invention has for its principal object the provision of a coating composition which, when applied to a suitable base material, will dry to a protective coating which simulates hammered metal in appearance.

Another object of this invention is to provide a coating technique which enables the production of a hammered metal finish by a one-coat application. This enables the rapid production of the finish and reduces the expense thereof to a considerable extent.

Other objects of this invention will more fully hereinafter appear.

This invention contemplates a method of application of the coating material by what is known as a one-coat practice. In this specification, the expression "one-coat" means that the coating composition is applied in one coat only and that no portion of the surface is gone over after the first coating on that portion has dried. As will presently appear, the term "one-coat" includes a method wherein the entire surface is gone over once and then, before any portion has dried, i. e. before the volatile solvent has had an opportunity to evaporate, the entire surface is gone over again so quickly that no portion of the first coat is allowed to dry or the volatile solvent contained therein allowed to evaporate before the second-coat is applied to that portion. The term "one-coat" also includes a method wherein the entire surface is gone over only once. This meaning of the term "one-coat" is a matter of common knowledge to those versed in coating methods.

I have discovered that by the application to a surface to be coated of a composition of matter comprising a synthetic or natural resinous base or varnish, metal powder and a thinner more fully described below, in such proportions as to form a sprayable coating composition by means of a spraying device so adjusted as to produce a spattering action, that a hammered metal finish is obtained by one coat.

As the base material to be provided with the hammered metal finish, I prefer to use any smooth, relatively hard surface such as metal, metal foil, regenerated cellulose sheets, wood, wood already lacquered or otherwise coated with a smooth, hard surface of enamel, varnish or the like, glass, ceramic ware, etc. However, I may apply my finishing material to fibrous materials such as cloth, woven fabrics, paper, and the like, after they have been provided with a smooth, hard surface of lacquer, or the like, which is not softened or dissolved excessively by the ingredients of my composition.

As the binder or base for my composition, I may use any natural or synthetic resinous base, such as a resin-oil varnish or the like. I may use either a natural or synthetic resin itself or I may use it dissolved in a drying oil to form a varnish base. As examples of suitable resins contemplated by this invention, I may enumerate phenol-formaldehyde or polybasic acid-polyhydric alcohol resins either unmodified or modified by numerous materials known in the art. These modifiers might include drying oils, drying oil fatty acids, non-drying oils, non-drying oil fatty acids, rosin, natural resins, such as copals, or such a resin as shellac. Any of the modified alkyd resins may have an additional phenol modification or treatment. Alternatively, I may use as a base cumarone-indene resin, reacted or cooked with a drying oil such as linseed oil. Similarly, other resins such as the phenol-aldehyde resins, copals, and other natural resins, may be cooked with an oil to produce a suitable base. The base may be either air-drying or of the type which is baked.

The base material may be either pigmented or unpigmented, as desired. In order, however, to produce a finish simulating more closely a genuine hammered metal finish, I find it highly desirable to have the base material pigmented by grinding it with a pigment designed to give an appropriate tint to the resulting finish. Thus, in the preferred practice of the invention, I use a black pigment in conjunction with aluminum bronze as the metallic powder whereby a black

hammered metal finish is obtained. Similarly, in producing a hammered copper finish I use a brown or pink pigment in conjunction with copper powder. In place of using a pigment to obtain the desired color in the finish, I may use dye-stuffs soluble in the coating composition. These and other modifications will be obvious to those skilled in the art. I may add the pigment or dye to the composition at any stage in its preparation, but I prefer to have it previously incorporated in the base material by grinding to form a synthetic enamel. I may ship the composition in three containers, the pigmented base or vehicle in one, the aluminum bronze in another and the unique thinner to be described below in the third, leaving it to the user to add the desired quantities of metallic powder (aluminum bronze) and thinner to the base immediately before use, or I may blend the complete composition together in the correct proportions and ship the finished product ready for application.

As the metal powder, I prefer to use aluminum powder in the form known to the art as "aluminum bronze." This is not a granular material, but consists of flakes. It is produced by a hammering process rather than by grinding. However, one may use copper, brass, bronze, gold or any other decorative, flake, metallic powder, although aluminum powder produces the best results because it tends to float readily on account of its low specific gravity, and because its color produces a closer simulation of a hammered metal effect than do the other powders enumerated. The finer this powder is the better results I am able to obtain. The powder must in any event be of such a fineness that it will have a tendency to float to the surface of the applied wet film. Stearic acid is commonly used as a lubricant in the production of metallic powder in the form of flakes, and is commonly present in small quantities in the commercial product. I have found that its presence is desirable. In some cases, I may add small amounts of stearic acid to my composition since it exerts a peculiar action upon the metal powder, increasing its floating tendency and improving the finish and producing greater uniformity of the hammered metal effect.

The thinner referred to above is composed of two miscible solvents of radically different volatilities, one of which is slowly volatile, known in the art as a high boiler, and the other of which is highly volatile, known in the art as a low boiler. As a preferred thinner, I use a mixture consisting of hydrogenated petroleum naphtha and denatured ethyl alcohol in the proportions of 33% of hydrogenated petroleum naphtha such as "Solvesso #3", having a flash point of 135° F. and boiling point range of 365-419° F., and 67% of denatured ethyl alcohol, having a flash point of 51.8° F. and a boiling point of about 172° F. As the denatured ethyl alcohol, I use an alcohol containing no undesirable denaturants which might spoil the finish and prefer to use specially denatured ethyl alcohol known as formula #1 which is denatured with about 5% of methyl alcohol, methyl alcohol being even more volatile than ethyl alcohol. The thinner contains the highly volatile solvent and the slowly volatile solvent in such proportions that if a plate of any smooth, hard material such as metal is coated with a thin film of the thinner alone and allowed to dry, the highly volatile solvent, in this case ethyl alcohol, will evaporate almost at once from the surface while the slowly volatile solvent,

namely the hydrogenated petroleum naphtha, will remain and will form into small individual droplets. The action of the thinner in the coating composition is to float the aluminum powder to the edge of these droplets as they are formed, giving rise to a great number of small circles and to the non-uniform effect known as a hammered metal finish.

It will be obvious that a thinner consisting of other solvents than those just described may be used, if desired. I may use any mixture of a slowly volatile solvent and a highly volatile solvent, which mixture will dissolve the resinous base material and form a suitable coating composition. The following solvent combinations may be used to produce variations in the hammered metal effect. Thus, in place of Solvesso No. 3, in conjunction with alcohol, I may use the same percentages of Solvesso No. 2 (boiling point range 275-365° F.), high flash petroleum naphtha, xylol, toluol, Solvesso No. 1 (boiling point range 200-275° F.), and similar slowly volatile solvents. In place of ethyl alcohol, I may use similar proportions of acetone, methyl alcohol, and similar highly volatile solvents. In general, the two solvents selected must be such that their boiling points have a difference of at least approximately 30° F. or more. Instead of using a single highly volatile solvent or a single slowly volatile solvent, I may use two or more solvents in each class. Where the claims specify "a solvent", such a mixture of two or more solvents, as well as a single solvent, is contemplated.

The thinner above described is added to the resinous base or vehicle at least in sufficient quantity to bring the same into solution, and preferably in considerable excess of this quantity for sprayability and so that greater opportunity is afforded for rapid evaporation of the highly volatile solvent by reason of the thus obtained lower proportion of total solids in the coating composition. The metal powder is added to the base either before or after the addition of the thinner. The mixture is shaken well, whereupon the metal powder is "floated", suspended or distributed throughout the solution. The coating composition is now ready for application.

A suitable quantity of the coating composition is placed into a pressure feed gun equipped with a spattering cap for the spray nozzle. However, any spray gun which will spatter is satisfactory. The method of application is such that the coating composition, by reason of the structure of the spraying device, is formed into relatively large individual droplets which are thrown onto the surface without substantial evaporation of any portion of the solvent contained therein during their projection from the spraying nozzle to the surface being coated. The pressure feed gun is connected with a source of air under pressure and is placed in operation at a suitable distance from the article to be finished which is gone over completely. The wet coated article dries very rapidly, forming the hammered metal effect almost immediately. It is then permitted to dry until hard or is baked if necessary to give it sufficient hardness.

For greater depth and thickness and for greater speed and uniformity, instead of employing the technique just described, I may first applying a "mist" of the coating composition just described over the entire surface of the work immediately following this before drying with a spattered coat of the same type just described. The fine drops from the mist form a uniform

coating over the entire surface which acts as a background for the spatter coat which is applied thereover. By a "mist", I refer to a fine spray obtained by adjustment of the spray gun in the correct manner.

As an example of a preferred coating composition contemplated by the present invention, I give the following:

A pigmented resinous base material is first prepared as follows:

The following ingredients in the following proportions are used—

|                    | Percent by weight |
|--------------------|-------------------|
| 15 Linseed oil     | 30                |
| Glycerine          | 35                |
| Phthalic anhydride | 35                |

Equal parts by weight of phthalic anhydride and glycerine are added into the kettle. This is heated slowly up to about 200°, at which point about half of the linseed oil is added. The mixture is heated very slowly up to 325° F. at which point the reaction, depending on the linseed oil composition, begins. The batch may be made up 25 in an inert atmosphere (such as carbon dioxide or nitrogen) and with or without mechanical agitation, but agitation is preferred. At 400° F. the remainder of the linseed oil is added and the temperature is increased to 425° F., and held 30 at this point until the reaction ceases. Then the temperature is raised to 450 or 460° F. until the right viscosity is obtained. The resin is then removed into a cooling kettle and allowed to cool. The foregoing in no way limits the resinous composition which may be used in this process. The alkyd base may be modified by other oils and acids; their amounts may be varied indefinitely, and an almost infinite variety of resinous compositions may be obtained by varying the percentages, kinds of ingredients, and the heating treatment. In the above resin, any color pigment may be ground in varying amounts, regulated by the color of the pigment, and its physical properties.

45 Any given quantity of the above described black, pigmented, resinous base material is taken. An equal volume of thinner composed of 33% by volume of hydrogenated petroleum naphtha in the form known as Solvesso No. 3 and 67% of 50 denatured ethyl alcohol, known as S. D. No. 1, is added to the pigmented resinous base material. The materials are agitated until a homogeneous solution is obtained. 4 ounces of finely divided 55 aluminum bronze powder are added to each gallon of the mixture. The solution or coating composition thus obtained produces, when spattered onto a smooth, hard, surface in the manner described above, a hammered metal finish having a marked resemblance to genuine hammered metal.

In the foregoing example, I am not limited as to the amount of bronze powder. It might run as low as 1/2 to 1 ounce per gallon or might be as much as 10 to 15 ounces per gallon, depending on the results which are desired.

It will be seen that I have devised a new coating composition and process of applying same of great usefulness in the art of finishing materials. It is to be understood that I do not wish to be limited to the specific description above but that this invention is to be limited only as set forth in the appended claims.

Having described my invention, what I claim is:

75 1. A coating composition adapted to produce

a hammered metal finish, said composition comprising a finely divided metal powder, a film-forming constituent consisting essentially of a material selected from the group consisting of synthetic and natural resins and synthetic and natural resin varnishes, and a solvent for the film-forming constituent in sufficient proportion to yield a fluid, readily sprayable mixture, said solvent consisting of a slowly volatile hydrogenated petroleum naphtha and a material selected from the group consisting of methyl alcohol, ethyl alcohol and acetone.

2. A coating composition adapted to produce a hammered metal finish which comprises a resinous base, a finely divided metal powder, and a solvent for the resinous base consisting of 33% of hydrogenated petroleum naphtha having a flash point of about 135° F., and a boiling point range of about 365-419° F., and of 67% of denatured ethyl alcohol having a flash point of about 51.8° F. and a boiling point of about 172° F.

3. A coating composition adapted to produce a hammered metal finish which comprises a mixture of equal volumes of a black, pigmented, synthetic resinous base and of a solvent for the same consisting of 33% of hydrogenated petroleum naphtha having a flash point of about 135° F. and a boiling point range of about 365-419° F., and of 67% of denatured ethyl alcohol having a flash point of about 51.8° F. and a boiling point of about 172° F., and aluminum bronze powder in the proportion of 4 ounces per gallon of said mixture.

4. A process of providing a base material with a finish simulating hammered metal which comprises applying thereto by a spattering operation a coating composition comprising a finely divided metal powder, a film-forming constituent consisting essentially of a material selected from the group consisting of synthetic and natural resins and synthetic and natural resin varnishes, and a solvent for the film-forming constituent in sufficient proportion to yield a fluid, readily sprayable mixture, said solvent consisting of a slowly volatile hydrogenated petroleum naphtha and a material selected from the group consisting of methyl alcohol, ethyl alcohol and acetone.

5. A process of providing a base material with a finish simulating hammered metal which comprises applying thereto by a spattering operation a coating composition comprising a resinous base, a finely divided metal powder, and a solvent for the resinous base consisting of 33% of hydrogenated petroleum naphtha having a flash point of about 135° F. and a boiling point range of about 365-419° F., and of 67% of denatured ethyl alcohol having a flash point of about 51.8° F. and a boiling point of about 172° F.

6. A process of providing a smooth, non-porous base material with a finish simulating hammered metal which comprises applying thereto by a spattering operation a coating composition comprising a mixture of equal volumes of a black pigmented synthetic resinous base and of a solvent for the same consisting of 33% of hydrogenated petroleum naphtha having a flash point of about 135° F. and a boiling point range of about 365-419° F., and of 67% of denatured ethyl alcohol having a flash point of about 51.8° F. and a boiling point of about 172° F. and aluminum bronze powder in the proportion of 4 ounces per gallon of said mixture.

7. A process of providing a metal surface with a finish simulating hammered metal which comprises applying thereto a mist of a coating com-

position which comprises a resinous base, a black pigment, finely divided aluminum powder and a solvent for the resinous base consisting of denatured ethyl alcohol and a slowly volatile hydrogenated petroleum naphtha, and then applying to said metal surface by a spattering operation the same material.

8. An article of manufacture comprising a smooth non-porous base material provided with a spattered surface film of a finishing material simulating hammered metal, said finishing material comprising the residue of a composition comprising a finely divided metal powder, a film-forming constituent consisting essentially of a material selected from the group consisting of synthetic and natural resins and synthetic and natural resin varnishes, and a solvent for the film-forming constituent in sufficient proportion to yield a fluid, readily sprayable mixture, said solvent consisting of a slowly volatile hydrogenated petroleum naphtha and a material selected from the group consisting of methyl alcohol, ethyl alcohol and acetone.

9. An article of manufacture comprising a smooth, non-porous base material provided with a surface film of a finishing material simulating hammered metal, said finishing material

comprising the residue of a composition comprising a resinous base, finely divided aluminum powder and a solvent for the resinous base in sufficient proportion to yield a fluid, readily sprayable mixture, said solvent consisting of 33% of hydrogenated petroleum naphtha having a flash point of about 135° F. and a boiling point range of about 365-419° F., and of 67% of denatured ethyl alcohol having a flash point of about 51.8° F. and a boiling point of about 172° F.

10. A process of providing a base material with a finish simulating hammered metal which comprises applying thereto a mist of a coating composition comprising a finely divided metal powder, a film-forming constituent consisting essentially of a material selected from the group consisting of synthetic and natural resins and synthetic and natural resin varnishes, and a solvent for the film-forming constituent in sufficient proportion to yield a fluid, readily sprayable mixture, said solvent consisting of a slowly volatile hydrogenated petroleum naphtha and a material selected from the group consisting of methyl alcohol, ethyl alcohol and acetone, and then applying to the mist-coated surface by a spattering operation the same material.

GUIDO ARIOTTI.